

J. SCHMITTINGER.  
DIAPHRAGM FOR THE SOUND BOXES OF TALKING MACHINES.  
APPLICATION FILED MAY 15, 1912.

1,104,833.

Patented July 28, 1914



Witnesses-

Charles H. York.  
Villa Bunnies.

Inventor  
John Schmittinger  
by his Attorneys-  
Howson & Howson

# UNITED STATES PATENT OFFICE.

JOHN SCHMITTINGER, OF PHILADELPHIA, PENNSYLVANIA, ASSIGNOR TO HOSMER W. HANNA, OF PHILADELPHIA, PENNSYLVANIA.

## DIAPHRAGM FOR THE SOUND-BOXES OF TALKING-MACHINES.

1,104,833.

Specification of Letters Patent.

Patented July 28, 1914.

Application filed May 15, 1912. Serial No. 697,534.

*To all whom it may concern:*

Be it known that I, JOHN SCHMITTINGER, a citizen of the United States, residing in Philadelphia, Pennsylvania, have invented 5 Improvements in Diaphragms for the Sound-Boxes of Talking-Machines, of which the following is a specification.

My invention relates to diaphragms for sound reproducing apparatus, more particularly the sound-boxes employed with talking machines; and the object of my invention is to provide an improved form of diaphragm designed to produce a softer tone than diaphragms heretofore employed 15 for the same purpose.

It is well known that it is impossible to obtain the best results with sound reproducing diaphragms made of the ordinary materials now in common use, such as metal, 20 paper, mica, &c., and while mica perhaps has gone into greater use than other materials, such diaphragms are extremely fragile and very expensive owing to the waste incident to the making of disks of 25 the proper size.

My improved diaphragm is made of an animal skin or integument treated in a peculiar and particular manner, which treatment results in the production of a 30 diaphragm capable, when employed as a reproducing agent in talking machine of the graphophone or phonograph type, of producing pleasing tones, avoiding the harshness and scratchiness common in the 35 use of many articles of this kind.

In the accompanying drawings, I have illustrated more or less diagrammatically the steps in the treatment of the material of which the diaphragms forming the subject of my invention are made, in which:

Figure 1, is a plan view of a skin from which the diaphragms are subsequently cut, showing the same before treatment; Fig. 2, is a view showing the treated skin mounted 45 in a stretching frame; Fig. 3, is a view of the finally treated skin, illustrating the cutting of the diaphragms therefrom; Fig. 4, shows the finished diaphragms, and Fig. 5, shows a pile of the finished diaphragms 50 weighted to insure maintenance of the same in a flat condition.

The material from which my improved diaphragms are made is that employed by banjo-makers for the banjo heads, being a 55 calf skin which has been tanned in a pecul-

iar manner to form what is technically known as "vellum." Of such skins, I prefer to use the portion taken from the back of the calf adjacent the backbone, and it is desirable that these skins be taken from calves as young as possible, preferably those new-born.

In some instances goat skins prepared for the same or similar purpose may be employed as the "raw" material from which my improved diaphragms are made.

In the drawings, 1 represents a skin in the condition received from the tanner. The skins thus procured are subjected to a bath consisting of about sixteen ounces of formaldehyde, (the usual 40% commercial solution of formic aldehyde), in which has been dissolved about one ounce of a suitable alkali, caustic potash (potassium hydrate), being preferred. The skins may be kept in such bath for a period of about 5 to 10 minutes, as may be necessary to effect substantially a retanning of the same and to soften them sufficiently to insure the desired stretching whereby they are increased in area and reduced in thickness. After this treatment, the skins are rinsed in cold water to remove all traces of the formaldehyde and caustic potash, and then they are placed in a suitable stretching frame 2, such as shown in Fig. 2 and dried.

When dry, the skins will be found to be much thinner, tougher, and substantially transparent, the original "raw" skin having been opaque; making ideal diaphragms. 90 They may be cut from the skin as illustrated in Fig. 3 by suitable means into the desired disks, as shown at 1<sup>a</sup> Fig. 4, which may be placed directly in the sound boxes, or packed away for further use. In the latter case they are preferably kept under more or less pressure as by means of a weight 5 to avoid warping or wrinkling.

In use there is no tendency of the diaphragms to swell or loosen, remaining perfectly taut, and in practice there seems to be some slight tendency to shrink; enhancing their vibratory qualities.

I claim:

1. A diaphragm for sound recording and reproducing machines, comprising a disk of previously tanned animal fiber hardened and toughened by the action of formaldehyde.

2. A diaphragm for sound recording and

reproducing machines, comprising a disk of previously tanned animal fiber hardened and toughened by the action of formaldehyde and caustic potash.

5 3. A diaphragm for sound recording and reproducing machines, comprising a disk of calf skin previously tanned to the form of vellum, hardened and toughened by the action of formaldehyde.

10 4. A diaphragm for sound recording and reproducing machines, comprising a disk of

calf skin previously tanned to the form of vellum, hardened and toughened by the action of formaldehyde and caustic potash.

In testimony whereof, I have signed my name to this specification, in the presence of two subscribing witnesses.

JOHN SCHMITTINGER.

Witnesses:

MURRAY C. BOYER,  
Jos. H. KLEIN.

Copies of this patent may be obtained for five cents each, by addressing the "Commissioner of Patents, Washington, D. C."